

## UNITED STATES PATENT OFFICE.

ALFRED EHRENREICH, OF LONDON, ENGLAND.

## PROCESS FOR OBTAINING TEXTILE FIBERS OF HIGH QUALITY FROM THE SKINS OF FISH SUCH AS, IN PARTICULAR, THOSE OF THE CHONDRopterygii-SELACHII.

No Drawing. Application filed January 24, 1928, Serial No. 249,205, and in Belgium January 27, 1927.

The subject of the invention is an improved process permitting of obtaining textile fibers of high quality from the skins of fish, especially those of the Chondropterygii-Selachii, and more particularly those of the sharks or Plagiostomi, the said process facilitating and thus rendering the treatment of the skins, with a view to obtaining textile fibers, more rapid and economical 10 and tending at the same time to the subsequent preservation of these fibers as well as to their improvement. The textile fibers obtained by the improved process cost less to produce, are very resistant, of a brilliancy 15 reminiscent of the lustre in silk and are of an excellent state of preservation, no matter what treatment they subsequently undergo.

This improved process is characterized by that:

20 1. After a short treatment with, for instance, lime, the fleshed skins are subjected to the diastasic action of enzymes, rendering it possible to disintegrate the skins.

It has been found that the skin of the 25 Chondropterygii-Selachii is very resistant to these diastasic actions and that, on the other hand, the intercellular substance is strongly decomposed and then finally destroyed by the enzymes, so that the adhesion between 30 the different fibers is reduced to such a degree that a slight mechanical treatment then suffices to obtain a fiber capable of being spun.

It is possible to use, for instance, trypsin, 35 i. e. the diastase of pancreatic sugar, either in the form of extracts or in the form of preparations with a basis of trypsin, such as, for instance, the product known as "oropone".

40 Instead of trypsin, it is possible to use extracts prepared from the glands of the Plagiostomi, such as sharks, and, in particular, the gland which is found at the commencement of the intestine, which corresponds to 45 the pancreas of the mammifera.

For instance, after the treatment with lime the skins are treated by means of an extract of trypsin or of shark glands for a period of 24 to 30 hours, at a temperature 50 varying between 35° and 40° C., the material and the liquid being, by preference, kept in a slight state of circulation.

2. After quickly rinsing the skins, the structure of which will be found to be

broken down, they are immediately subject- 55 ed to the tanning process by means of any suitable tanning agents, vegetable, mineral or artificial. The trypsin decomposes the intercellular substance, thus decreasing the cohesion between the different fibers and 60 thus breaking down the structure of the skin as stated. Owing to this treatment the fibers acquire a fixed brilliancy comparable with that of silk and are permanently protected from the causes of deterioration or 65 destruction.

3. After the skins are tanned, they are dried and then defibered, the separation of the constituent fibers being effected, by preference, mechanically, for instance by being 70 passed through carding and opening machines similar to those used in the carding of wool or cotton waste. The fibers so obtained permit of the manufacture of fabrics, the brilliancy of which is comparable with 75 that of silk and which are extremely resistant and capable of being printed, dyed, dressed or otherwise treated, without the fibers being in any way altered by such treatment.

With the object of facilitating the disintegration of the skins and the subsequent defibering, it has been found advantageous immediately after the treatment of the skins by the enzymes, to treat them with certain 80 colloids, preferably with colloids of the nature of gum tragacanth, such as, for instance, tragasol.

Obviously it is possible, without departing from the invention, to apply variations and 90 modifications in details of the process forming the subject thereof, for instance the tanning process, instead of being applied to the skins before defibering, could be applied to the fibers themselves.

What I claim is:

1. An improved process for obtaining textile fibers of high quality from the skins of fish such as those of the Chondropterygii-Selachii and more particularly those of the Plagiostomi such as sharks, characterized in that the fleshed skins after a short treatment with lime are disintegrated by being subjected to the diastasic action of enzymes, the said skins then being rinsed, tanned, dried and defibered either by hand or mechanically by any suitable known appliance, substantially as described.

2. An improved process for obtaining textile fibers as claimed in claim 1, characterized in that the skins after being subjected to the diastasic action of enzymes are rinsed, dried and defibered either by hand or mechanically by any suitable known appliance the fibers produced being tanned in any suitable way, substantially as described.
3. An improved process for obtaining textile fibers as claimed in claim 1, characterized in that the skins are disintegrated by the diastasic action of trypsin either in the form of extracts or of preparations such as, for instance, oropone, substantially as described.
4. An improved process for obtaining textile fibers as claimed in claim 1, character-

ized in that the disintegration of the skins is effected by the diastasic action of the liquid secreted by the pancreatic glands of the *Plagiostomi*, substantially as described.

5. An improved process for obtaining textile fibers as claimed in claim 1, characterized in that the disintegrated skins immediately after the treatment with enzymes or the equivalent are treated with colloids such as tragasol, substantially as described.

6. A textile fiber of high quality obtained from the skins of fishes such as *Chondropterygii-Selachii* and in particular of *Plagiostomi* or sharks.

In testimony whereof I affix my signature.

ALFRED EHRENREICH.